

# UNITED STATES PATENT OFFICE.

SUMNER SIMPSON, OF BRIDGEPORT, CONNECTICUT, ASSIGNOR TO RAYBESTOS COMPANY,  
A CORPORATION OF CONNECTICUT.

## PROCESS OF MAKING FRICTION-FACINGS.

1,301,612.

Specification of Letters Patent. Patented Apr. 22, 1919.

No Drawing.

Application filed May 22, 1918. Serial No. 236,055.

*To all whom it may concern:*

Be it known that I, SUMNER SIMPSON, a citizen of the United States, residing in the city of Bridgeport, county of Fairfield, and 5 State of Connecticut, have invented certain new and useful Improvements in Processes of Making Friction-Facings, of which the following is the specification.

This invention relates to improvements in 10 process of making friction facings and refers more particularly to the clutch facings and brake linings for motor vehicles and the like.

Among the salient objects of the present 15 invention are to provide a process of making a friction facing from unwoven short felted asbestos fiber, the fiber being united into a compact and uniform mass by means of a comminuted binder; to provide a process 20 of the character referred to in which a uniform wearing surface is provided formed from short asbestos fiber; to provide a process which permits of the use of a short asbestos fiber, thus utilizing as far as the 25 weaving is concerned a substantially waste product; to provide an improved method of saturating a friction facing and in such a way as to insure the uniform and complete saturation of the ring by the comminuted 30 binder, and in general to provide an improved process of the character referred to.

In the co-pending application I have claimed a friction facing made of unwoven felted asbestos fiber, and the present invention 35 relates to the economical process of manufacturing the same. As is well known to those skilled in the art the mine run of asbestos consists of relatively long fibers and relatively short fibers. The long fibers are 40 the only portion that can be utilized for spinning and weaving. Heretofore long fiber asbestos has been utilized in the manufacture of woven clutch facings. This woven asbestos friction facing consists essentially of wire covered with asbestos and 45 then woven to form a friction facing. In the manufacture of annular friction facing, such as clutch rings, it has been the practice to stamp or cut the ring out in straight strips 50 and then unite the ends by a suitable joint. This has been necessary for the reason that in stamping rings out of the woven sheet the greater part of the sheet would of course be waste, as far as making any further rings 55 are concerned. Inasmuch as the remainder

of the sheet cannot thereafter be used to make rings it was not practical to stamp out the rings. In the present invention, however, the rings can be stamped out without resulting waste for the reason that that part 60 of the sheet left after the rings are stamped out can be again re-used to make a new sheet.

Describing now the means of carrying out the process, the asbestos fiber is first ground in a suitable crusher or grinding machine and is then put into a beater and mixed with water or other liquid solution and beaten into a pulp. The pulp is then treated to a further water bath and finally delivered to the paper making machine and 65 formed into laminated sheets of suitable 70 width and thickness. From there the sheet passes through suitable presses and driers.

Preferably this sheet is of sufficient width to permit of four or more friction facings 75 being stamped or cut out of its width. In the manufacture of clutch facings of the ring or annular type they can be easily and readily stamped out of the body of the sheet. This, of course, obviates the necessity of the 80 jointed ring. The clutch facings of the cone type can be also formed. Where the endless ring facings are formed it is, of course, apparent that after they are stamped out of the sheet the larger part of the sheet is left 85 from which no further rings can be formed. This waste material has then to be placed 90 into a grinder and beater and run through the process as before to form a new batch. The economy and simplicity of this operation is its chief merit. By this process in time the entire material of the original sheet will finally be formed into clutch rings. No such economy and efficiency of operation 95 can be approximated in the woven rings if endless unjointed ring facings are to be formed. After the rings are stamped out or linings, if it is desired to make linings, they are then impregnated or saturated with the desired binder. Various binders are 100 used. However, the question of satisfactorily impregnating or saturating the friction facing has offered practical difficulties. One difficulty results, not from the inability 105 of the binder to perform its function when once it is thoroughly saturated into the facing, but in obtaining a sufficient saturation of the facing. The binder may consist of a hard asphalt, natural or artificial, mixed with a suitable oil, as a vegetable or a min- 110

eral oil, and then this mixture thinned with a suitable vehicle, such as gasolene or benzene. I have further discovered that the manner in which this mixture is made has 5 an important effect on the saturating ability of the mixture. Take, for example, a mixture of gilsonite, linseed oil and gasolene, much more efficient results are obtained by first mixing the melted gilsonite and linseed 10 oil thoroughly together and then adding the gasolene or other vehicle. This produces more efficient results than where all three are mixed simultaneously. While this manner of mixing the binder seems relatively 15 simple, it took considerable experimenting to ascertain just how this should be done. After the friction members are saturated with the binder, as above stated, they may be subjected to a heated air treatment if desired. It is also to be understood that the 20 friction facings may be pressed down to a micrometer thickness.

The invention is not limited to the details above shown except as set forth in the appended claims.

25

I claim as my invention:

1. A process of making friction facings which consists in forming an asbestos facing, mixing a hard bitumen with a suitable oil by melting the bitumen into the oil and then adding to this mixture a volatile vehicle, and finally saturating the facing with a binder formed as above stated.

2. A process of making friction facings which consists in making a friction facing, 35 mixing gilsonite, or the like, with a vegetable oil such as linseed oil, by melting the gilsonite and mixing it with the oil and then adding to such mixture a volatile vehicle such as gasolene, and finally impregnating 40 the facing with this binder formed as above stated.

SUMNER SIMPSON.